

(No Model.)

B. MOEBIUS.

# PROCESS OF AND APPARATUS FOR SEPARATION OF METALS.

No. 532,209.

Patented Jan. 8, 1895.

FIG. 1.



ప్రార్థన.



Fig. 4.



**WITNESSES:**

WITNESSES.

INVENTOR:  
Bernard Moebius,  
BY  
*Amberdampf*  
ATTORNEY

THE NORRIS PETERS CO., PHOTO-LITHO., WASHINGTON, D. C.

# UNITED STATES PATENT OFFICE.

BERNARD MOEBIUS, OF NEW YORK, N. Y.

## PROCESS OF AND APPARATUS FOR SEPARATION OF METALS.

SPECIFICATION forming part of Letters Patent No. 532,209, dated January 8, 1895.

Application filed February 28, 1894. Serial No. 501,854. (No model.)

*To all whom it may concern:*

Be it known that I, BERNARD MOEBIUS, a citizen of the United States, and a resident of New York, in the county and State of New York, have invented certain new and useful Improvements in Processes of and Apparatus for the Separation of Metals, of which the following is a specification.

My invention relates to an improved method and apparatus for separating metals by electrolysis, its principal object being to withdraw the silver or other deposited metal from the apparatus as fast as it is deposited and to prevent short circuiting caused by the formation of bridges between the anodes and cathodes.

For this purpose my invention consists essentially in passing the cathode through the bath in close proximity to the anode or anodes, depositing the silver on the cathode in a loose, spongy or crystalline form, collecting the silver carried off by the cathode and discharging it continuously outside of the bath and preventing the anions and cations from being mixed with each other.

In carrying out my invention I use by preference apparatus of the nature shown in the annexed drawings, in which—

Figure 1 is a sectional elevation of the apparatus, part being broken away. Fig. 2 is a vertical cross-section on the line  $x-y$ , Fig. 1; Fig. 3, a detail view of the contact lever for the anodes. Fig. 4 is a detail view showing modified forms for the diaphragm and frame.

Referring now to the drawings the letter A represents a tank of the usual construction for the electrolytic bath.

B, B' are rolls placed within the tank, one of which, B, is rotated in the direction of the arrow by suitable means, such as the pulley P.

C is an endless apron stretched between the rolls B and B' and supported by intermediate rolls b, b'. This endless apron is the cathode and is for this purpose formed entirely of sheet metal, by preference silver, or it may be made of sheet metal with a non-metallic backing; or of non-metallic material upon one side of which a coating of silver is de-

posited by electrolysis and firmly compressed during the process of deposition; or copper may first be deposited and then coated with silver. As seen in the drawings, the entire endless cathode is contained within the bath and is stretched horizontally.

E, E are frames and G anode plates supported by said frames E. The bottom of the frames consists of diaphragms of muslin or other suitable material such as porous earthenware, or the whole frame together with the bottom may be a dish of porous earthenware as shown in Fig. 4 where E', G' is the porous dish. The frames E are removably supported upon the sides of the tank A.

D is an endless apron or conveyer formed of rubber cloth, canvas, or other suitable material. It is stretched between rolls d and d', the roll d being rotated in the direction of the arrow by suitable means, such as the chain n and wheels N and O.

K is a conductor, supplied with positive current from a dynamo-machine, and connected with the anodes G (formed of the bullion to be separated), by contact arms M.

L is the conductor for the negative current connected with the movable cathode C by brushes F. The contact arms M are by preference made of copper and the ends protected by rubber sleeves r and thin platinum caps m, as shown in Fig. 3.

S is a scraper bearing against the lower part of the apron D, and R a receptacle into which the silver or other deposit is discharged. The receptacle R is provided with a strainer for filtering off the liquid carried over with the deposit.

The bullion to be separated is cast into anode plates G which are placed into the frames E so as to be immersed in the exciting liquid and the anions and cations are thus separated by the diaphragms and prevented from being mixed. As an exciting liquid I use by preference a strong solution of sodium or potassium nitrate sufficiently acidulated with nitric and sulphuric acid to keep some silver and all the copper in solution, such a bath being a very good conductor of electricity.

When parting bullion containing silver, gold, copper, and other metals, a current of small electromotive force is used, and the dissolved silver is precipitated upon the cathode 5 C in a loose spongy state or in crystalline form. It is slowly carried by the cathode C over the roll B and either collected in the tank near its end, whence it may be removed, or by preference collected upon a conveyer D, which at 10 once takes it out of the tank and discharges it into the receptacle R, whence it is taken to the melting pot. The copper is dissolved but remains in solution, provided the exciting liquid be properly acidulated and not too poor 15 in silver and too rich in copper.

By slowly moving the cathode past the anodes, collecting the deposit therefrom and again presenting fresh surfaces of the cathode to the anodes, short circuiting, such as generally 20 caused by bridges formed between the anodes and cathodes, is prevented. The cathode may pass very close to the anodes, thus reducing resistance. The crystals deposited upon the cathode form part of the same, increasing 25 the surface and likewise reduce resistance. The work goes on continuously without interruption for cleaning. The silver is delivered ready for the melting pot, instead of being blocked up in the apparatus and requiring 30 the investment of large capital.

The apparatus is very simple and requires but little repair and attention.

The gold and the platinum metals are retained upon the diaphragms, together with 35 lead peroxide, some peroxide of silver and other impurities. Whenever any one of the anode plates is exhausted its contact lever is raised up and a fresh anode plate put in. The residue upon the diaphragms is collected in 40 rotation, so that there is no interruption in the process. This residue, containing gold and other metals is treated in the usual well known manner.

By the method and apparatus described the 45 entire anode is subjected to the action of the current, and no scraps are left, which have to be remelted as in other processes.

While the method and apparatus above described are designed particularly for separating 50 alloys containing silver, they may be used for other purposes, as for instance for the electrolytic deposition of copper in a loose, spongy state.

By arranging a series of vats in tiers one 55 above the other and discharging all the silver into one and the same receptacle, a great economy in space may be effected.

What I claim as new is—

1. The herein described method of refining 60 alloys containing silver, which consists in placing the alloys as anodes into a bath suitable for dissolving silver and copper therefrom, subjecting the anodes to an electric current of small electromotive force; slowly passing 65 a silver cathode through the bath beneath the

anodes and in close proximity to the same, preventing the mixing of anions and cations, depositing the silver upon the cathode in a loose, spongy, or crystalline form, and collecting the silver deposited on the cathode, substantially as specified. 70

2. The herein described method of refining alloys containing silver, which consists in placing the alloys as anodes into a bath suitable for dissolving silver and copper therefrom; subjecting the anodes to an electric current of small electromotive force, slowly passing a silver cathode through the bath beneath the anodes and in close proximity to the same; preventing the mixing of anions and cations, 75 depositing the silver in a loose, spongy or crystalline form upon the cathode and continuously carrying the same out of the bath by mechanical means, substantially as specified. 80

3. The herein described method of refining alloys containing silver, which consists in placing the anodes into a bath of nitrates sufficiently acidulated to keep the copper in solution; subjecting the anodes to an electric 90 current of small electromotive force, slowly passing a cathode through the bath beneath the anodes and in close proximity to the same, preventing the mixing of anions and cations, depositing the silver upon the cathode in a 95 loose spongy or crystalline form, leaving the gold, platinum metals and impurities at the anodes, collecting the silver from the cathode and discharging it, substantially as specified. 85

4. The herein described method of refining alloys containing silver, consisting in subjecting the alloy as anode to an electric current of small electro motive force in a bath of an alkali nitrate, such as sodium nitrate, sufficiently acidulated with nitric and sulphuric 105 acid to keep the copper in solution, passing a cathode of silver through the bath beneath the anodes and in close proximity to the same, depositing the silver upon the cathode in a loose spongy or crystalline form, collecting it 110 and carrying it out of the bath, and preventing the mixing of the anions and cations, substantially as specified. 100

5. In an electrolytic apparatus for the separation of metals, the combination of an anode 115 formed of the metals to be separated, a horizontal endless cathode in the form of an endless apron, diaphragm frames suitable for receiving and submerging anode plates, placed horizontally in close proximity to the upper 120 part of the endless cathode and adapted to prevent the mixing of anions and cations, and mechanical means for collecting the deposit from the endless cathode, substantially as described. 125

6. An electrolytic apparatus consisting of the vat A, anode frames E with diaphragms, 130 endless cathode C stretched on rolls, means for slowly moving the endless cathode beneath the anodes and in close proximity to 135

the same; proper electric connection for the anodes and the cathode and a conveyer adapted to collect the deposit from the endless cathode within the bath and to deliver it 5 outside the bath, substantially as specified.

In testimony that I claim the foregoing as my invention I have signed my name, in pres-

ence of two witnesses, this 24th day of February, 1894.

BERNARD MOEBIUS.

Witnesses:

A. FABER DU FAUR, Jr.,  
KLAS H. TERNSTEDT.